# EUROPEAN PATENT SPECIFICATION

(11) **EP 3 061 867 B1**
(45) Date of publication and mention of the grant of the patent: **12.06.2019**
(21) Application number: 14856708.4
(22) Date of filing: 23.10.2014
(51) Int. Cl.: E01B 1/00, E01C 3/00

(54) **BALLAST AND METHOD FOR PRODUCING SAME**
SCHOTTER SOWIE VERFAHREN ZU DESSEN HERSTELLUNG
BALLAST ET PROCÉDÉ DE SON OBTENTION

(30) Priority: 23.10.2013 ES 201331557
(43) Date of publication of application: 31.08.2016
(73) Proprietor: Universitat Politècnica De Catalunya, 08034 Barcelona (ES); Comsa S.A.U., 08014 Barcelona (ES); Mapei S.p.A., I-20158 Milano (IT); Administrador de Infraestructuras Ferroviarias, 28020 Madrid (ES)
(72) Inventor: LÓPEZ PITA, Andrés, 08034 Barcelona (ES); MANZO COSTANZO, Nahuel, 08028 Barcelona (ES); FONTSERÈ, Valentí, 08023 Barcelona (ES); AUSILIO, Antonio, 20096 Pioltello (Mi) (IT); DE AMBRI, Emanuele, 20017 Rho (Mi) (IT); BASEI, Elisa, 20068 Peschiera Borromeo (Mi) (IT)
(74) Representative: Juncosa Miró, Jaime
(86) International application number: PCT/ES2014/070798
(87) International publication number: WO 2015/059335

(56) References cited:
- WO-A1-2010/119123
- WO-A1-2011/031168
- WO-A1-2011/131621
- WO-A1-2011/131621
- WO-A1-2013/120059
- WO-A1-2013/120059
- AT-B- 405 424
- DE-A1- 3 712 461
- DE-A1- 19 632 639
- ES-A1- 2 356 964
- ES-T1- 2 167 289
- FR-A1- 2 202 978
- FR-A1- 2 553 445
- JP-A- H10 279 340
- RU-C1- 2 447 220
- RU-C1- 2 447 220
- DATABASE WPI Week 200337, Derwent Publications Ltd., London, GB; AN 2003-384803, XP055334853 RETRIEVED & JP 2002 326225 A (MISAWA TOYO CO LTD) 12 November 2002
- DATABASE WPI Week 200814, Derwent Publications Ltd., London, GB; AN 2008-B87498, XP055334858 RETRIEVED & JP 2008 019630 A (RAILWAY TECHNICAL RES INST ET AL.) 31 January 2008
- DATABASE WPI Derwent Publications Ltd., London, GB; XP055334863 RETRIEVED: 'BALLAST PRISM FOR HIGH-SPEED HEAVY-TRAFFIC SECTIONS OF CONTINUOUS WELDED RAILROAD TRACK' & RU 2011 114322 A (G OBRAZOVATEL NOE UCHREZHDENIE VYSSHEGO PROFESSIONAL NOGO OBRAZOVANIJA) 20 October 2012
- DATABASE WPI Week 199602, Derwent Publications Ltd., London, GB; AN 1996-017696, XP055334875 RETRIEVED & JP H07 292 603 A (KOWA KASEI) 07 November 1995

## Description

### Field of the Art

The present invention relates to a ballast with improved characteristics in terms of durability and resistance to fragmentation with respect to other rail track bed materials.

The invention also relates to the method for producing said improved ballast. State of the Art

The use of ballast as a rail track bed is widely known, but it has some drawbacks.

First, the aggregate suitable for this use must meet required characteristics which are more exacting the higher the speed of the trains is or the higher the load that said trains transport, the sharpness of the edges of the aggregate being one of the essential characteristics, because said sharpness is what provides stability and prevents the ballast from flowing and causing track deformations with train vibrations. The difficulty in finding aggregates that meet all the characteristics required by sets of technical specifications makes them more expensive and leads to the need to move them over great distances, making them even more expensive.

Another problem lies in the fact that vibrations to which the ballast is subjected due to the passage of trains cause the aggregates to become rounder over the years and to lose qualities, leading to the need of costly maintenance tasks or to the reduction in track performances.

Furthermore, vehicles circulating at high speed often cause the aggregates to be lifted off the ballast and pelted against the undersides of the train, being able to cause malfunctions.

Some products and methods for mitigating these drawbacks are known, such as for example, the invention described in patent document WO2011131621A1, where it anticipates the use of a ballast layer impregnated with a component which is subsequently sprayed with a second component producing a reaction, generating a protective polyurethane layer binding the ballast and prolonging its service life, but at the expense of complicating its maintenance or replacement, in addition to achieving an excessively monolithic result, greatly reducing the elasticity of the assembly. It must also be pointed out that the application of said chemical components *in-situ* can cause environmental contamination problems. WO 2013/120059 A1 further discloses a crushed ballast consisting of aggregates individually coated with a polymer layer that integrates a granular elastomer material.

Another known alternative is the use of a polymer as an individual coating for each aggregate, as described in the document entitled "Characterization of polyurethane coated railroad ballast behavior", presented in the 90th Annual Meeting of the Transportation Research Board, Washington, DC in January 2011. This solution prevents the contamination problems of the *in-situ* application of the ballast polymer coating, but the faces of the stones remain flat, without any relief that improves binding.

Finally, the use of granular particles of an elastomer material is also known, such as for example, through patent document DE102007053146A1, describing the mixture of small particles of an elastomer material between the ballast to provide it with certain elasticity and to improve the adherence between the aggregates. The problem with this embodiment is that vibrations tend to stratify the components of the ballast, and said granules of the elastomer material can come out of the ballast very easily and contaminate the track surroundings.

### Brief Description of the Invention

The proposed invention relates to a crushed ballast with improved durability and resistance to fragmentation for rail infrastructures, consisting of aggregates with a particle size distribution selected from between 25 mm and 100 mm, individually coated with a first solidified polymer layer which integrates a granular elastomer material with granules having a size smaller than 4 mm, preferably having a size smaller than 2 mm.

These granules of the elastomer material are fixed on the surface of the aggregates by means of the solidification of the polymer material and allow increasing in a remarkable manner the roughness of the aggregate as they confer protuberances to said aggregate. Said protuberances provide an improved binding of the aggregates with one another as a result of their increased roughness, due to the simple geometric interference of said protuberances and to the higher coefficient of friction of these materials compared to the aggregate, whereby the total resistance and durability of the ballast is increased, in addition to its overall stability against vibrations.

Furthermore, by arranging elastomer granules between the aggregates, the vibrations can be absorbed by these granules, without causing the mentioned aggregates to wear out at all, such that the service life of the ballast is prolonged along with its elasticity, making it unnecessary to arrange elastomer parts between the ties and the ballast or between the tracks and the ties. A reduction in the noise level produced by the passage of trains as well as a reduction in the ballast-flying phenomenon as the train passes are also achieved. Furthermore, an aggregate treated accidentally pelted against the undersides of the train would cause less damage as it is coated with an elastomer material.

According to the invention, it is proposed to arrange a second polymer layer over the aggregate provided with the elastomer material adhered with the first polymer layer, said second polymer layer providing a protective coating for protecting the elastomer material, and an increased fixing.

This arrangement allows using aggregates which, before receiving the proposed coating, do not have the characteristics required for use thereof as a rail ballast, either because their edges are not sharp enough, or because of another reason. Old and worn-out ballasts, or aggregates discarded from a quarry, or recycled construction materials, or quarry ballasts that do not meet the strict requirements established by the standards for use thereof as a rail track ballast, for example by standard UNE EN 13450 2003, can therefore be used, for example. This and other similar standards greatly limit the type of aggregates that can be used, but the proposed coating increases the properties of the initial aggregate, whereby an aggregate which initially did not comply with said standard or another standard can be treated such that, after treatment, it indeed complies with said standard and can be used, thereby widening the range of stones which can be used as raw material, being able to use materials that are much more economical and easy to find than conventional aggregate. This also allows having closer supply sources and reducing logistics costs.

The granular elastomer material can originate from the shredding of recycled material, such as for example, tires, which increases the value of highly polluting waste, and allows giving it a new use, in addition to taking advantage of its properties with a competitive cost.

Optionally, the polymer material will be a material from the polyurethane family, since its elasticity and resistance properties, as well as its drying process and compatibility with other raw materials that are contemplated make it an optimal material, allowing it to be applied in liquid form and to solidify quickly. Furthermore, once the drying process is completed no pollutants are discharged to the environment.

The method applied for producing the ballast object of the present invention consists of applying in liquid form the first polymer layer on the aggregate. This method can be carried out, as a non-limiting example, by means of spraying or pouring a polymer product on an aggregate which is spread on and conveyed by a flush grid conveyor belt, or by means of immersing said aggregate into a tank containing said polymer material, and it is then extracted and dispersed so that it can be dried in the crushed form, by means of a vibrating conveyor, for example.

According to a first non-limiting embodiment, the granular elastomer material can be integrated to the aggregate by means of mixture thereof with the liquid polymer material before the application thereof on the aggregate, or according to a second embodiment, it can be adhered to the aggregate already impregnated with the polymer material but before drying same, for example by means of scattering or pouring the said elastomer material on the aggregate, this aggregate being spread on a flush grid conveyor belt or on a vibrating conveyor. Another possibility of application of the elastomer material is by means of immersion by means of vibration of the aggregate impregnated with the polymer material before drying same in a tank filled with said granular elastomer material.

In a non-limiting illustrative manner, the polymer material can be of the type which solidifies in contact with moisture, or by evaporation of volatile fractions, or by heat drying, or as it reacts upon applying a second component, in this case the method described up until now would be followed by the application of this second component to trigger solidification.

According to the invention, the inclusion of a second coating polymer layer has been envisaged to assure the complete adhesion of the elastomer material to the aggregate. This second layer can be applied in a way similar to the way the first layer is applied.

This method of treating aggregate for producing the proposed ballast can be developed by means of a treatment plant having a small enough size so as to allow transport by road or by train to a location close to the location where the ballast must be installed. This possibility again reduces the production costs as transport of the raw materials is reduced.

### Brief Description of the Drawings

The foregoing and other advantages and features will be better understood based on the following detailed description of an embodiment which must be interpreted in an illustrative and non-limiting manner in reference to the attached drawings in which the sizes of the granules of the elastomer material as well as the thickness of the coatings have been expressly emphasized, in which:
Figure 1 shows a section of an aggregate on which a first polymer layer has been applied, a plurality of granules of the elastomer material were adhered to said first polymer layer before the solidification thereof;
Figure 2 shows a section of the same aggregate shown in Figure 1 on which a second polymer layer has been applied to strengthen the fixing of the granules;
Figure 3 shows a section of an aggregate on which a first polymer layer consisting of a mixture of said polymer product with the granules of the elastomer material has been applied, these granules being embedded in said first layer;
Figure 4 shows a section of the same aggregate shown in Figure 3 on which a second polymer layer has been applied to strengthen the fixing of the granules; and
Figure 5 shows a schematic view of the ballast formed by a plurality of the aggregates shown in any one of the first four figures, showing how the geometric interference of the granules of the elastomer material confers greater stability to the assembly.

### Detailed Description of an Embodiment

As can be seen in the attached Figures 1 to 4, the proposed coating for aggregates 1 allows producing aggregates provided with protuberances. These protuberances, when putting a plurality of these aggregates 1 in a heap to form a ballast base for a railway track, generate a geometric interaction between these protuberances, greatly increasing the stability of the assembly (Figure 5).

Figure 1 shows an aggregate which has been coated with a first polymer layer 2 on which the granules of the elastomer material 3 have been adhered, Figure 2 shows this same configuration but provided with a second polymer layer 4 strengthening the fixing of the elastomer material 3.

Figure 3 shows an aggregate which has been coated with a first polymer layer 2 that had been previously mixed with the granules of the elastomer material 3 which have adhered to the aggregate 1 upon applying said first polymer layer 2. Figure 4 shows this same configuration but provided with a second polymer layer 4 strengthening the fixing of the elastomer material 3. These added protuberances thereby allow increasing the stability of the assembly, being able to use as raw material aggregates which would have been dismissed for use thereof as ballast, due to them not having sufficient binding properties and resistance, normally due to them not having sharp enough edges or being too rounded. This insufficiency is compensated for by the added protuberances. Furthermore, it allows greater irregularity of the particle size distribution of the ballast, since the cohesion of the assembly no longer depends on the correct interaction between the edges of the aggregates. This characteristic allows using as raw material for producing the proposed ballast more economical materials that are more easily accessible than the conventional materials, such as for example, old, worn-out recycled ballast, aggregates which have not passed the tests required for use thereof as ballast, construction rubbles, aggregates with a particle size distribution not acceptable for use thereof as conventional ballast, aggregates with rounded edges, etc.

The mentioned protuberances being of an elastomer material allows, in addition to a high stability, the ballast to have certain elastic properties and to be capable of absorbing vibrations without wearing out. This property results in greater durability, less frequent maintenance, a lower noise level as the train passes, and an increased safety.

Said elastomer material 3 can be formed completely or partially by rubber originating from shredded tires, an economical material which constitutes increasing the value of waste.

The production method used in the aggregates 1 shown in Figures 1 and 2 consists of, only by way of non-limiting example, conveying the aggregates 1 scattered on a conveyor belt on which there are arranged application means applying the first polymer layer 2 on the aggregates 1. Said impregnated aggregates 1 are then introduced in a tank containing said granular elastomer material 3. A plurality of granules is randomly adhered to the outer face of each aggregate 1 because the first polymer layer 2 has still not solidified. Said aggregates 1 are then extracted from said tank, and the first polymer layer 2 is then solidified. Said process will depend on the selected polymer, and may include steps of timed drying, heat drying, or application of a reactive component. This step can optionally be followed by the application and solidification of the second polymer layer 4.

In the case of the aggregates shown in Figures 3 and 4, the production process can consist of, by way of non-limiting example, a step of mixing the granular elastomer material 3 with the polymer material, for then pouring the mixture on a flush grid conveyor belt conveying the aggregates 1, the first polymer layer 2 and the elastomer material 3, thereby being applied simultaneously to proceed to the solidification thereof and to the optional application of the second polymer layer 4.

## Claims

1. A crushed ballast for rail infrastructures consisting of aggregates (1) with a particle size distribution selected from between 25 mm and 100 mm, individually coated with a first solidified polymer layer (2), wherein said first polymer layer (2) integrates a granular elastomer material (3); **characterized in that** a second solidified polymer layer (4) is arranged individually coating each aggregate (1) and the corresponding first polymer layer (2) integrating the mentioned granular elastomer material (3).

2. The ballast according to claim 1, **characterized in that** the size of the granules of the elastomer material (3) is smaller than 4 mm.

3. The ballast according to claim 1 or 2, **characterized in that** at least part of the aggregate (1) used is a recycled aggregate.

4. The ballast according to claim 3, **characterized in that** at least part of the aggregate (1) used is an aggregate selected from the following: recycled worn-out ballast, construction rubbles, low-quality quarry ballast, or ballast with a particle size distribution less than 40 mm.

5. The ballast according to any of claim 1 to 4, **characterized in that** at least one part of said granular elastomer material (3) is a recycled material originating from shredded tires.

6. The ballast according to any one of the preceding claims, **characterized in that** at least one of said polymer layers (2, 4) is made from polyurethane.

7. A method for producing a crushed ballast for rail infrastructures, the method providing an individual coating to aggregates (1) with a particle size distribution selected from between 25 mm and 100 mm with at least a first polymer layer (2) integrating a granular elastomer material (3),
**characterized in that** it comprises
a first step which comprises adding to an aggregate (1) a first polymer layer (2) in a solidifiable liquid form integrating an elastomer material: and a second step which comprises adding a second polymer layer (4) in a solidifiable liquid form onto said first polymer layer (2) and granular elastomer material (3).

8. The method according to claim 7, **characterized in that** said second polymer layer (4) is added after the solidification of the first polymer layer (2).

9. The method according to any one of claims 7 to 8, **characterized in that** said granular elastomer material (3) is mixed with the liquid polymer material forming the first polymer layer (2) before application thereof on the aggregate (1).

10. The method according to any one of claims 7 to 8, **characterized in that** said granular elastomer material (3) is added to said aggregate (1) after the application of the first liquid polymer layer (2) and before the solidification thereof.

11. The method according to any one of claims 7 to 10, **characterized in that** an aggregate (1) at least partially recycled is used.

12. The method according to any one of claims 7 to 11, **characterized in that** at least one part of said granular elastomer material (3) used is a recycled material originating from shredded tires.

13. The method according to any one of claims 7 to 12, **characterized in that** the granules of the elastomer material (3) used have a size smaller than 4 mm.

## Patentansprüche

1. Zerkleinerter Schotter für Eisenbahninfrastrukturen bestehend aus Zuschlagstoffen (1) mit einer Partikelgrößenverteilung ausgewählt aus zwischen 25 mm und 100 mm, einzeln mit einer ersten verfestigten Polymerschicht (2) beschichtet, wobei die genannte erste Polymerschicht (2) ein granulöses elastomeres Material (3) integriert; **dadurch gekennzeichnet, dass** eine zweite verfestigte Polymerschicht (4) derart angeordnet ist, dass sie jeden Zuschlagstoff (1) einzeln beschichtet und die entsprechende erste Polymerschicht (2) das genannte granulöse elastomere Material (3) integriert.

2. Schotter nach Anspruch 1, **dadurch gekennzeichnet, dass** die Größe der Granulate des elastomeren Materials (3) kleiner als 4 mm ist.

3. Schotter nach Anspruch 1 oder 2, **dadurch gekennzeichnet, dass** mindestens ein Teil des verwendeten Zuschlagstoffes (1) ein recycelter Zuschlagstoff ist.

4. Schotter nach Anspruch 3, **dadurch gekennzeichnet, dass** mindestens ein Teil des verwendeten Zuschlagstoffes (1) ein Zuschlagstoff ist, ausgewählt aus den Folgenden: einem recycelten abgenutzten Schotter, Bauschutt, Bruchsteinschotter niedriger Qualität oder Schotter mit einer Partikelgrößenverteilung kleiner als 40 mm.

5. Schotter nach einem der Ansprüche 1 bis 4, **dadurch gekennzeichnet, dass** mindestens ein Teil des genannten granulösen elastomeren Materials (3) ein recyceltes Material ist, welches aus geschredderten Reifen stammt.

6. Schotter nach einem der vorhergehenden Ansprüche, **dadurch gekennzeichnet, dass** mindestens eine der genannten Polymerschichten (2, 4) aus Polyurethan hergestellt ist.

7. Verfahren zur Herstellung eines zerkleinerten Schotters für Eisenbahninfrastrukturen, wobei das Verfahren eine einzelne Beschichtung auf Zuschlagstoffen (1) mit einer Partikelgrößenverteilung ausgewählt aus zwischen 25 mm und 100 mm mit mindestens einer ersten Polymerschicht (2), welche ein granulöses elastomeres Material (3) integriert, bereitstellt, **dadurch gekennzeichnet, dass** es Folgendes umfasst:
einen ersten Schritt, welcher das Hinzufügen zu einem Zuschlagstoff (1) einer ersten Polymerschicht (2) in einer verfestigbaren Flüssigform, welche ein elastomeres Material integriert, umfasst; und
einen zweiten Schritt, welcher das Hinzufügen einer zweiten Polymerschicht (4) in einer verfestigbaren Flüssigform auf der genannten ersten Polymerschicht (2) und dem granulösen elastomeren Material (3), umfasst.

8. Verfahren nach Anspruch 7, **dadurch gekennzeichnet, dass** die genannte zweite Polymerschicht (4) nach der Verfestigung der ersten Polymerschicht (2) hinzugefügt wird.

9. Verfahren nach einem der Ansprüche 7 bis 8, **dadurch gekennzeichnet, dass** das genannte granulöse elastomere Material (3) mit dem flüssigen Polymermaterial, welches die erste Polymerschicht (2) bildet, vor dem Auftragen derselben auf dem Zuschlagstoff (1) gemischt wird.

10. Verfahren nach einem der Ansprüche 7 bis 8, **dadurch gekennzeichnet, dass** das genannte granulöse elastomere Material (3) zum genannten Zuschlagstoff (1) nach dem Auftragen der ersten flüssigen Polymerschicht (2) und vor der Verfestigung derselben hinzugefügt wird.

11. Verfahren nach einem der Ansprüche 7 bis 10, **dadurch gekennzeichnet, dass** ein mindestens teilweise recycelter Zuschlagstoff (1) verwendet wird.

12. Verfahren nach einem der Ansprüche 7 bis 11, **dadurch gekennzeichnet, dass** mindestens ein Teil des genannten verwendeten granulösen elastomeren Materials (3) ein recyceltes Material ist, welches aus geschredderten Reifen stammt.

13. Verfahren nach einem der Ansprüche 7 bis 12, **dadurch gekennzeichnet, dass** die Granulate des verwendeten elastomeren Materials (3) eine Größe kleiner als 4 mm aufweisen.

## Revendications

1. Ballast en pierre concassée pour infrastructures de rail consistant en des agrégats (1) ayant une distribution de taille de particule sélectionné entre 25 mm et 100 mm, revêtue individuellement d'une première couche de polymère solidifié (2), dans lequel
cette première couche de polymère (2) intègre un matériau élastomère granuleux (3) ; **caractérisé en ce qu'**une deuxième couche de polymère solidifié (4) est aménagée revêtant individuellement chaque agrégat (1) et la première couche de polymère correspondante (2) intégrant ce matériau élastomère granuleux (3).

2. Le ballast conformément à la revendication 1, **caractérisé en ce que** la taille des granules du matériau élastomère (3) est inférieure à 4 mm

3. Le ballast conformément à la revendication 1 ou 2 **caractérisé en ce qu'**au moins une partie de l'agrégat (1) utilisé est un agrégat recyclé.

4. Le ballast conformément à la revendication 3, **caractérisé en ce qu'**au moins une partie de l'agrégat (1) utilisé est un agrégat sélectionné des suivants : ballast usé recyclé, gravats de construction, ballasts de carrière de faible qualité ou ballast ayant une distribution de particule inférieure à 40 mm

5. Le ballast conformément à une quelconque des revendications 1 à 4, **caractérisé en ce qu'**au moins une partie de ce matériau élastomère granuleux (3) est un matériau recyclé provenant de pneus déchiquetés.

6. Le ballast conformément à une quelconque des revendications précédentes, **caractérisé en ce qu'**au moins une de ces couches de polymère (2,4) est faite de polyuréthane.

7. Une méthode pour fabriquer un ballast en pierre concassée pour infrastructures de rail, la méthode offrant un revêtement individuel aux agrégats (1) ayant une distribution de taille de particules sélectionnée entre 25 mm et 100 mm ayant au moins une première couche de polymère (2) intégrant un matériau élastomère granuleux (3),
**caractérisée en ce qu'**elle comporte
une première étape qui comporte ajouter à un agrégat (1) une première couche de polymère (2) sous fourme de liquide solidifiable intégrant un matériau élastomère ; et
une deuxième étape comportant ajouter une deuxième couche de polymère (4) sous une forme liquide solidifiable à cette première couche de polymère (2) et matériau élastomère solidifiable (3).

8. La méthode conformément à la revendication 7, **caractérisée en ce que** cette deuxième couche de polymère (4) est ajoutée après la solidification de la première couche de polymère (2).

9. La méthode conformément à une quelconque des revendications 7 à 8, **caractérisée en ce que** ce matériau élastomère granuleux (3) est mélangé avec le matériau de polymère liquide formant la première couche de polymère (2) avant son application sur l'agrégat (1).

10. La méthode conformément à une quelconque des revendications 7 à 8, **caractérisée en ce que** ce matériau élastomère granuleux (3) est ajouté à cet agrégat (1) après l'application de la première couche de polymère liquide (2) et avant sa solidification.

11. La méthode conformément à une quelconque des revendications 7 à 10, **caractérisée en ce qu'**un agrégat (1) au moins partiellement recyclé est utilisé.

12. La méthode conformément à une quelconque des revendications 7 à 11, **caractérisée en ce qu'**au moins une partie de ce matériau élastomère granuleux (3) utilisé est un matériau recyclé provenant de pneus déchiquetés.

13. La méthode conformément à une quelconque des revendications 7 à 12, **caractérisée en ce que** les granules du matériau élastomère (3) utilisé ont une taille inférieure à 4 mm.
